

C. A. PFANSTIEHL.  
TUNGSTEN CONTACT POINT.  
APPLICATION FILED APR. 6, 1914.

1,220,886.

Patented Mar. 27, 1917.



*Witnesses:*

Robert F. Brucke  
Leonard E. Bogue

Inventor  
Carl A. Efanstiehl  
By Brown, Williams, Bell, Hausner & Gottsche  
Attorneys

# UNITED STATES PATENT OFFICE.

CARL A. PFANSTIEHL, OF WAUKEGAN, ILLINOIS, ASSIGNOR TO PFANSTIEHL COMPANY,  
A CORPORATION OF DELAWARE.

## TUNGSTEN CONTACT-POINT.

1,220,886.

Specification of Letters Patent. Patented Mar. 27, 1917.

Application filed April 6, 1914. Serial No. 830,013.

To all whom it may concern:

Be it known that I, CARL A. PFANSTIEHL, a citizen of the United States, residing at Waukegan, in the county of Lake and State of Illinois, have invented certain new and useful Improvements in Tungsten Contact-Points, of which the following is a full, clear, concise, and exact description, reference being had to the accompanying drawings, forming a part of this specification.

My invention relates to a process for the production of tungsten electrical contacts and to the particular type of contact point produced by such process.

Metallic tungsten is one of the group of so-called rare metals. It fuses only at extremely high temperatures. It does not readily oxidize or corrode in ordinary atmospheres. It is extremely hard, and can not be cut or worked with ordinary tools. Its properties are such as to make it admirably adapted for electrical contact points of electrical switching mechanisms of various types, but the high cost for the metal itself, coupled with the difficulties in working it into shape for use, has greatly limited if not indeed practically prevented its application as a material from which to make electrical contact points.

The process of my invention involves the cutting of appropriate disks of tungsten from the end of a rod whose cross-section corresponds substantially to that of the finished contact points. The tungsten disk thus made is preferably attached to a base metal stem by means of a film or layer of gold, silver or copper fused or welded both to the base metal stem and the tungsten of the contact point proper.

I have found that disks of tungsten cut or ground from the end of a worked or drawn tungsten rod in the manner herein-after described are far preferable for the purposes of electrical contacts to disks which are stamped or punched from a sheet of tungsten, the reason being that the fiber or grain of a sheet of metallic tungsten is parallel with the surface of the sheet so that the

side of the grain or fiber is subjected to the wear of the contact points as mounted in 50 electrical switching mechanism. In a tungsten rod, on the other hand, the grain is lengthwise of the rod and the disks cut from the end thereof, by the process hereinafter described, present the end of the grain of the 55 tungsten as the contact circuits with the result that the wear upon the point is far more uniform than in the case of disks cut from sheet metal.

I have found also that the contact points 60 thus cut from the end of a rod are far less subject to pitting due to the arcing to which switch contact points are subjected than are points punched from sheet tungsten and that the latter crumble away at the edges, where- 65 as there is little or no crumbling at the edge of my contact points when used under similar conditions.

The process of carrying out my invention as embodied in the machine for doing it, and 70 the tungsten rod before being cut and disk after being cut, are illustrated in the accompanying drawings in which like characters designate like parts throughout, and in which,

Figure 1 illustrates the grinding or slitting machine by means of which the disks are cut from the end of a tungsten rod;

Fig. 2 illustrates a disk of tungsten;

Fig. 3 illustrates the disk of silver by 80 means of which the disk of tungsten is fused to the head of the mounting stem shown in Fig. 4.

Referring first to Fig. 1, I have illustrated a rod of tungsten 20, which is preferably 85 of circular cross-section and of the diameter of the finished contact point. This tungsten rod is inserted in a closely-fitting hole 21 of the clamping frame 22, the clamping mechanism being provided with a movable 90 clamping member 23 provided with a screw-threaded rod 24 upon which the clamping nut 25 may be turned to clamp the tungsten rod 20 in the end of the clamping member, as shown.

The clamping member is provided with a

2  
gage 26, the thickness of the end 27 of the gage being approximately that of the tungsten disks to be cut from the end of the rod. A stop 28 is pivotally mounted at 29, whereby the adjustable screw 30 in the end of the stop lever may be swung down to the position shown in the drawings to serve as an abutment to stop the movement of the rod 20 when the rod is pushed to the right 10 through the hole in the clamping member. The handle 31 may be depressed to raise the screw 30 from its normal position opposite the hole through the gage member 26.

The entire clamping mechanism as thus far described is mounted upon a carriage 15 adapted to slide in a T-shaped slot 32 formed in the base of the cutting machine. A rack 34 mounted upon the carriage co-operates with a pinion 35 to advance the carriage 20 with its clamping mechanism whenever the operating lever 36 is manipulated, the motion being transmitted through the crank arm 37, which is provided with a pin 38 riding in the slot 39 of the lever 36, which 25 in turn is pivoted at 40, as illustrated.

Mounted upon the common base plate 41 is the rotatable spindle 42 of the grinding head, provided with rollers or ball bearings mounted in the frame 43. A belt runs over 30 the pulley 44 to rotate the spindle 42, upon the end of which is mounted the slitting wheel 45. This slitting wheel is preferably not much more than one one-hundredth of an inch in thickness, and I support it between the metal disks 46 and 47, these disks 35 extending near but not quite to the periphery of the slitting wheel 45.

The slitting wheel is rotated at high speed to cut the disks from the end of the tungsten rod 20. The operation of this part of the mechanism employed in carrying out my process involves the adjustment of the rod of tungsten within the clamping mechanism, as shown in the drawings, whereupon the 40 lever 36 is manipulated to force the end of the rod of tungsten against the periphery of the slitting wheel. The pressure is continued until the wheel has cut or ground its way through the tungsten. The tungsten disk 45 thus cut from the end of the rod is retained in the hole in the end 27 of the gage 26 until the side of the slitting wheel has passed entirely across the face of the disk, as a result of which the bur which would otherwise 50 be formed at one side of the tungsten disk is entirely removed. When a disk has thus been cut from the end of the rod the carriage is withdrawn, due to the pull of the retracting spring 48. Thereupon, the handle 31 of the stop mechanism is depressed to permit the finished tungsten disk to drop from the hole in the end 27 of the gage 55 piece 26. The nut 25 is then turned to the

left to loosen the clamping mechanism, whereupon the tungsten rod 20 may be 60 pushed to the right until it engages the screw 30 of the stop mechanism. The nut 25 is then tightened to clamp the rod firmly in position, whereupon it is ready for another slitting or cutting operation. 70

The slitting wheel 45 is formed of carborundum grain, alundum grain or preferably a mixture of both, rolled or otherwise formed in a sheet of an unvulcanized mixture of rubber gum and sulfur. This sheet 75 containing the carborundum grain or crystals is then vulcanized to form a hard vulcanite wheel in which the grain or crystals are firmly embedded. I have found it preferable to employ carborundum dust of from 80 60 to 100 mesh, and I have found it desirable also to add to the unvulcanized rubber mixture a sufficient percentage of sodium silicate to assure the production of a hard and tough wheel after the vulcanizing operation has been performed. 85

The vulcanite carborundum wheels above described may be made extremely thin and can be satisfactorily operated without breaking when held between clamping disks, as 90 shown in Fig. 1, and provided also that the spindle upon which the wheel is mounted is provided with closely-adjusted bearings, and provided also that the entire mechanism is so strongly and firmly constructed 95 as to avoid chatter or vibration.

After the tungsten disks are cut from the end of the rod as above described, they must be thoroughly cleaned and freed from any film of oxid. This is done by treating the 100 disks in a hot bath of solution of caustic potash or soda, whereupon they are ready to be mounted upon the clean stems of base metal such, for example, as iron or steel. A stem such as I prefer to employ is illustrated in Fig. 4, the head, somewhat like the head of a nail, being shown at 50 and the shank being indicated at 51. These stems are preferably made of iron or steel sufficiently soft to permit the insertion of the 110 shank 51 through the hole of a contact spring or lever, whereupon the shank may be riveted to secure the stem and its tungsten contact face securely in place. 105

While I have described my invention in 115 connection with the use of tungsten disks, I do not wish to be limited to the use of pure tungsten, for the reason that tungsten alloyed with certain other rare metals can advantageously be substituted for pure tungsten. Small percentages of molybdenum, for example, may be alloyed with the tungsten with results in some instances better than those secured from the use of substantially pure tungsten. 120 125

I do not wish, therefore, to be limited to

the precise details herein described, but claim as my invention:

1. A make and break electrical contact of drawn tungsten in which the grain or fiber of the tungsten extends perpendicularly to the contact face.

2. An electrical make and break contact sawed from the end of a tungsten rod, so that the fiber or grain of the tungsten ex-

tends perpendicularly to the impact face of 10 the contact.

In witness whereof, I hereunto subscribe my name this 24th day of March, A. D. 1914.

CARL A. PFANSTIEHL.

Witnesses:

A. G. McCaleb,  
ALBIN C. AHLBERG.